

Aug. 25, 1942.

E. J. DUNN

2,293,972

MANUFACTURE OF STEEL CASTINGS

Filed Feb. 13, 1941

LEGEND:

— COM. NO. 1

— COM. NO. 2

— DUKITE



*Inventor:*

EDWARD J. DUNN  
by: John E. Jackson  
his Attorney

## UNITED STATES PATENT OFFICE

2,293,972

## MANUFACTURE OF STEEL CASTINGS

Edward J. Dunn, Duquesne, Pa.

Application February 13, 1941, Serial No. 378,810

4 Claims. (Cl. 22—216)

This invention relates to the manufacture of metallic ingots and, particularly, to an improved means for covering the molten metal in the tops of ingot molds to effect an insulation and exothermic condition.

In the usual practice of casting steel ingots, the molten metal is taken from the furnace in a liquid state and carried in a ladle, from which it is poured into ingot molds generally made of cast iron of a square, rectangular, or round section to form ingots which afterwards are shaped in rolling mills to commercial products. The steel in cooling and solidifying in these molds will, of course, shrink, and solidification will start immediately after the steel is poured and comes in contact with the inner walls of the mold.

In such practice, the top of the metal freezes over, leaving a large shrinkage cavity under the surface and, as a result, when the ingot thus formed has finally cooled there will be, due to this shrinkage of the steel, a cavity commonly known as a "pipe" in the top central part of the ingot of substantially a conical shape tapering toward the bottom. The surface of this "pipe," when exposed to the atmosphere after the pouring has been completed, becomes oxidized and this part of the ingot will not, in the process of rolling or forming into a commercial product, be welded solidly into a homogeneous mass with the rest of the ingot and, consequently, the end of the ingot, on the dead head or crop, as it is sometimes called, containing such pipe must be discarded as scrap; thus, clearly reducing the usable portion of the ingot.

Various means have been employed to reduce the pipe and increase the recoverable part of the ingot, but none of them have proved to be very satisfactory. One of the methods most commonly used is to place on top of the ingot mold a hot top, which is either a hollow tile or a cast iron box lined with a suitable refractory material. The purpose of such a hot top is, of course, to retain the temperature of the poured liquid steel as long as possible so that the steel in the upper part of the ingot remains molten for a time after the outside of the ingot in contact with the mold walls solidifies, thus tending to fill the shrinkage cavity in the center of the ingot to shorten the length of the pipe. While the use of the hot top as a means of insulating the molten metal has been effective, it has not shortened the "pipe" to any great extent nor increased the usable portion of ingots.

Furthermore, when the top of the molten metal solidifies and the freezing proceeds downwardly 55

in the mold, the carbon and other elements in the metal tends to segregate, which is, of course, undesirable in that it reduces the quality of the ingot and the steel.

5 The present invention relates to a means for preventing excessive shrinkage and piping of the ingot and excessive segregation of the metal as it solidifies, so as to provide an ingot which is sounder and free from pipe and segregation of carbon and other elements, thereby producing a higher yield of ingot to finished product.

Accordingly, it is one of the objects of my invention to provide an improved exothermic covering means for the top of the molten metal in an ingot mold so as to prevent excessive shrinkage of this part of the ingot as it solidifies, and an insulating means which maintains the metal molten for a predetermined length of time.

It is another object of the invention to provide 20 an improved exothermic covering means for the top of the molten steel in an ingot mold so as to prevent excessive segregation of the carbon and other elements, whereby a better ingot is produced having an extremely high yield.

25 It is a further object of this invention to provide an improved exothermic covering means for the top of the molten steel in ingot molds having an ash content related to the carbon content of the steel with which it is used.

30 It is still another object of the invention to provide an improved exothermic covering means for the top of the molten metal which is simple and inexpensive and, at the same time, one which is efficient and effective in its use.

35 Various other objects and advantages of my invention will become more apparent during the course of the following specification and appended claims.

The improved means of my invention for insulating molten metal in the tops of ingot molds 40 consists of dry anthracite coal which I have named "Dukite." The anthracite coal is preferably in the form of finely ground anthracite slack which is divided into various grades, according 45 to its ash content. River coal (dried), being a low grade, fine anthracite coal which is recovered from rivers by dredging, it having been run into the river during the washing process of anthracite lump coal, is very practical for use, but 50 it will be understood that anthracite coal from any other source is satisfactory.

It has been found that the dry anthracite coal or "Dukite," when applied to the top surface of the molten metal in an ingot mold, acts as an insulation and causes an exothermic reaction

which maintains the steel in the hot top molten for a considerable length of time, thus affording a more efficient feeding of the molten metal down into the shrinkage cavity which forms as the ingot solidifies. The feeding of the molten metal with the use of "Dukite" results in substantially a reduced U-shaped cavity where a V-shaped cavity normally occurs. It also has been found by comparison that dry anthracite coal of various grades of ash content, in the manner as it is proposed to be used according to the present invention, provides ingots with a far greater yield than ingots using other types of insulating means.

The dry anthracite coal or slack is classified preferably into six grades, according to the ash content, as follows:

- Grade No. 1—having an ash content up to approximately 16 per cent;
- Grade No. 2—having an ash content of from approximately 16 to 19 per cent;
- Grade No. 3—having an ash content of from approximately 19 to 23 per cent;
- Grade No. 4—having an ash content of from approximately 23 to 26 per cent;
- Grade No. 5—having an ash content of from approximately 26 to 28 per cent; and
- Grade No. 6—having an ash content in excess of 28 per cent.

It has been found that grades Nos. 1, 2 and 3 of "Dukite," that is, anthracite coal having an ash content up to approximately 23 per cent, are satisfactory for use with low carbon steel, namely, steel having a carbon content up to approximately 0.14 per cent; that grades Nos. 1, 2, 3, and 4, that is, coal having an ash content up to approximately 26 per cent, are satisfactory for use with medium carbon steel, namely, steel having a carbon content of approximately 0.40 per cent; and that all six grades, that is, coal having an ash content up to and in excess of 28 per cent, are satisfactory for high carbon steels, namely, steels having a carbon content of approximately 0.96 per cent. The proper grade of anthracite coal or "Dukite" for steels having a carbon content in between or above those given can be conveniently found by experimentation.

The following conventional procedure for casting an ingot is employed, with which the insulating means of the present invention is used. The molten metal is carried from the furnace in a ladle in a manner well known to those skilled in the art, from which the molten metal is poured into the ingot molds. After the proper amount of molten metal has been poured into any particular mold, according to the present invention the proper grade of dry anthracite coal or "Dukite" is applied loosely to the top surface thereof. The particular grade of anthracite coal or "Dukite" used is selected according to its ash content, with the ash content thereof depending upon the carbon content of steel being poured into the molds and with which it is to be used. It is preferable that the grades hereinbefore mentioned for steels having corresponding carbon content be used. The anthracite coal or "Dukite," when disposed upon the top of the molten metal, will tend to distribute itself uniformly over the entire top surface thereof so as to provide an insulating and exothermic blanket thereon, thereby insulating the same. As the main body of the ingot solidifies, the metal in the hot top and in the top portion of the mold is maintained liquid due to this insulating blanket of anthracite coal or "Dukite," thus affording more opportunity for a denser and less segregated ingot. It will be

understood that my insulating means may be used with or without a hot top, but it is preferable that a hot top be used, as better results will be obtained.

It has been found that by selecting the correct grade of anthracite coal; that is, one having an ash content in an amount which is related to the carbon content of the metal, that the top portion of the ingot will remain molten the proper length of time sufficiently long to obtain the maximum benefits in the elimination of piping and segregation and not too long so as to hold back production. For the average size ingot a grade of "Dukite" is selected so that the metal remains molten for a period of about one hour and a half, which is just about the proper length of time to obtain the maximum benefits therefrom so as to produce an ingot satisfactory in all respects.

In order to ascertain the advantages of the use of the insulating means or "Dukite" of my invention over the use of other insulating means, experiments have been made and it has been compared with other types of insulating materials. To illustrate the results of these experiments, there is shown in the drawing a graph illustrating the effect of the use of anthracite coal or "Dukite" on carbon segregation, in which the abscissa represents the inches below the hot top junction in the ingot, and the ordinate represents the percentage in variation from the ladle carbon analysis in hundredths of one per cent. In this graph the segregation of the carbon in an ingot with the use of the insulating means or "Dukite" (Grade No. 3) of my invention is compared with the segregation of carbon in ingots where two commercial types of insulating materials were used, these two insulating materials being ones which have given the highest yield of any known commercial coverings heretofore used. It is common practice, a fact which is well known to those skilled in the art, that steel having more than a 10-point variation of carbon from the ladle analysis, that is, more than .10 per cent variation, is unsatisfactory for use and generally discarded, and that when no insulating means is used, the hot top and about 10 inches below the hot top junction must be discarded, due to the segregation of the carbon in the upper portion of the mold and in the hot top. Referring to the graph, it will be seen that with the use of the two commercial insulating materials or covers, the hot top and about 4 inches below the hot top junction must be discarded. However, it will be seen that with the use of anthracite coal or "Dukite," according to my invention, that only the metal in the hot top need be discarded, due to the fact that the metal below the hot top junction is within the 10-point variation. Thus, it will be seen that with the use of my insulating means there is considerable savings in metal and there is also considerably less variation in carbon from the ladle analysis, thereby at the same time increasing the quality of the ingot.

It has been found through quite extensive experimentation with several ingots that when a grade of anthracite coal or "Dukite" having an ash content up to approximately 23 per cent is used for insulating steel having a low carbon content (approximately 0.14 per cent carbon), that the average midway carbon variation from the ladle analysis was 0.025 per cent; that the average center carbon variation from ladle analysis was 0.036 per cent; and that with the use of anthracite coal having an ash content of over 23

per cent, the average midway carbon variation was 0.036 per cent and the average center variation was 0.074 per cent. Thus, it will be seen that in the low carbon steels the carbon variation was much less in the use of anthracite coal having a low ash content (less than 23 per cent) than with the use of coal having a higher ash content (over 23 per cent).

With the use of a grade of anthracite coal or "Dukite" having an ash content up to 26 per cent for insulating steel having a medium carbon content (approximately 0.40 per cent) it was found that the average midway carbon variation from the ladle analysis was 0.042 per cent; that the average center carbon variation from the ladle analysis was 0.058 per cent; and that with the use of anthracite coal having an ash content in excess of 26 per cent, the average midway variation was 0.039 per cent and the average center variation, 0.138 per cent. Thus, it will be seen that in the medium carbon steel, the carbon variation was much less in the use of anthracite coal having a low ash content (less than 26 per cent) than with the use of coal having a high ash content (over 26 per cent).

With the use of any grade of anthracite coal for insulating high carbon steel (approximately 0.96 per cent), it was found that the average midway carbon variation from the ladle analysis was 0.020 per cent and that the average center carbon variation was 0.060 per cent. Accordingly, it will be seen that it is important that a grade of anthracite coal having the proper ash content be used, in order to obtain an ingot having the least carbon variation. That is to say, the anthracite coal used for insulating should be selected in view of the carbon content of the particular steel with which it is adapted to be used. Therefore, it will be seen that the ash content of the anthracite coal is critical with respect to the carbon content of the steel.

While the insulating means or "Dukite" of my invention may be used without the use of a refractory hot top, the benefits derived therefrom are not as pronounced as if a hot top were used.

As a result of my invention, it will be seen that there is provided an improved and inexpensive means for insulating the molten metal in the tops of ingot molds which reduces and practically eliminates the pipe in the top of the ingot and at the same time reduces segregation of the carbon and other elements in the steel to a minimum, thereby producing an ingot having a greater yield and one of much better quality. With the use of the insulating material of my invention, it has been found that the yield of an ingot is as much as 90 per cent, which is much greater than the yield obtained by the use of any other insulating means.

From the above description of my invention, it will be apparent that many modifications of the

same may be devised within the scope thereof and all such modifications are contemplated as may fall within the scope of the appended claims.

I claim:

- 5 1. In the manufacture of metallic castings, the method of casting the same which comprises pouring the molten metal into a mold, selecting a dry anthracite coal in the form of slack having an ash content in an amount which is related to the carbon content of the metal, and applying said slack loosely to the top surface of the molten metal so as to provide a uniform insulating blanket over the entire top surface thereof, whereby excessive piping and excessive segregation of the metal is prevented.
- 10 2. In the manufacture of steel castings, the method of casting the same which comprises pouring the molten metal into a mold, selecting a dry anthracite coal in the form of slack having an ash content in an amount related to the carbon content of the steel, said slack having an ash content up to approximately 23 per cent for steel having a carbon content of approximately 0.14 per cent, and an ash content up to approximately 26 per cent for steel having a carbon content of approximately 0.40 per cent, and applying said slack loosely to the top surface of the molten steel so as to provide a uniform insulating blanket over the entire top surface thereof whereby excessive piping and excessive segregation of the steel is prevented.
- 15 3. In the manufacture of steel castings and the like, the method of casting the same which comprises pouring the molten metal into a mold, selecting a dry anthracite slack having an ash content of a predetermined amount and in relation to the carbon content of the steel being cast with said slack having an ash content of up to approximately 26 per cent for steel having a carbon content of approximately 0.40 per cent, and applying said slack loosely to the top surface of the molten metal so as to provide a uniform insulating blanket over the entire top surface thereof whereby excessive piping and excessive segregation of the metal is prevented.
- 20 4. In the manufacture of steel castings and the like, the method of casting the same which comprises pouring the molten metal into a mold, selecting a dry anthracite slack having an ash content in an amount which is related to the carbon content of the steel being cast, said slack having an ash content up to and in excess of 28 per cent for steel having a carbon content in excess of approximately .40 per cent, and applying the said slack loosely to the top surface of the molten metal in the mold so as to provide a uniform insulating blanket over the entire top surface thereof whereby excessive piping and excessive segregation of the metal are prevented.
- 25
- 30
- 35
- 40
- 45
- 50
- 55
- 60

EDWARD J. DUNN.